

## UNITED STATES PATENT OFFICE.

CHARLES E. LAVERTY, OF PITTSBURG, PENNSYLVANIA; ARTHUR F. LAVERTY ADMINISTRATOR OF SAID CHARLES E. LAVERTY, DECEASED.

## PICKLING-BATH.

No. 856,644.

Specification of Letters Patent.

Patented June 11, 1907.

Application filed August 28, 1905. Serial No. 276,165

*To all whom it may concern:*

Be it known that I, CHARLES E. LAVERTY, of Pittsburg, county of Allegheny, and State of Pennsylvania, have invented a new and 5 useful Improvement in Pickling-Baths, of which the following is a full, clear, and exact description.

My invention relates to the pickling of metal for the purpose of removing scale or 10 oxid from its surface preparatory to further treatment such as coating the metal by galvanizing or tinning.

The object of my invention is to provide a 15 pickling-bath, by the use of which the time necessary to remove the scale or oxid from the surface of the metal treated is greatly reduced, and in the use of which the scale or oxid is removed from the metal without appreciably attacking the surface of the metal.

Another object of my invention is to provide a pickling-bath in the use of which, the 20 weight of metal lost in pickling is reduced from about 3 per cent., as is lost by the ordinary pickling solutions in use, to about 4 25 of 1 per cent.

My invention consists in the mixture of a hydrocarbon with the sulfuric acid ordinarily used in such pickling operations.

In the preparation of the pickle in its preferred form, I first add a hydrocarbon to what is known as 30 degree sulfuric acid, the materials being mixed in a suitable vat. Tar sludge is the material preferably used containing the hydrocarbon, on account of its 35 cheapness, it being a waste product of the oil refining process, containing tar, oil and sulfuric acid although oil or other forms of hydrocarbons may be used. I preferably add the sludge to the acid generally about 1 part 40 sludge to 15 parts acid by weight. This will give an excess of oil to the acid, the surplus oil being afterward skimmed from the top of the bath.

In preparing the pickling solution for shipment, in order to save weight, it is made of 45 much greater strength than is required for use and by its subsequent addition to water

the solution is diluted to the required degree of strength for use.

The mixture is constantly agitated while 50 being mixed and when an acid of less strength is used, the mixture may be heated by means of heat, externally applied to the vat, or by a steam jet introduced into the vat. After the materials are thoroughly mixed they are 55 allowed to stand for some time, when the excess hydro-carbon rises to the top of the solution when it is then skimmed off and the solution is ready for use. The mixture of acid and oil which is of much greater strength 60 than required for use after the excess oil has been removed by skimming, is then added to a sufficient amount of water, until the solution has a specific gravity of about 3 to 15 degrees Baumé. While adding the solution of 65 acid and oil to the water, the materials are thoroughly mixed by stirring or preferably by means of a steam and air jet introduced by a suitable pipe into the mixing vat.

The advantages of my invention lie in providing a pickling bath, by the use of which, the time required for removing the scale from the surface of the metal treated is greatly reduced and in which the surface of the metal is not attacked by the acid in the bath to any 75 appreciable extent during the time required to remove the scale from the metal.

By the use of the improved pickling-bath, the amount of material required to subsequently coat the metal treated is greatly reduced, there being practically no decomposed metal on the surface of the pickled material, to be burned off and form dross and sal-ammoniac skimmings in the coating bath, as is the case in the usual process. The 85 surface of the pickled material is finished smooth and in this way also the amount of coating material required is reduced.

Variations in the materials used and in the proportions of the materials used may be 90 made without departing from my invention.

Other than sulfuric acid may be used and materials other than oils containing hydrocarbon may be combined with the acid, since

What I claim is:—

1. A pickling-bath containing a hydrocarbon.
2. A pickling-bath containing an acid and a hydrocarbon.
3. A pickling-bath containing sulfuric acid and with a hydrocarbon.
4. A pickling bath containing an acid and a hydrocarbon oil.

5. A pickling bath containing sulfuric acid and a hydrocarbon oil.

In testimony whereof, I have hereunto set my hand.

CHARLES E. LAVERTY.

Witnesses:

R. D. LITTLE,  
GEO. B. BLEMING.